

Mar. 6, 1923.

1,447,218

E. J. LOWRY

PLOWSHARE

Filed Feb. 24, 1921



E. J. Lowry Inventor  
By Seymour & Bright  
Attorneys

Patented Mar. 6, 1923.

1,447,218

# UNITED STATES PATENT OFFICE.

EDMUND JAMES LOWRY, OF SOUTH BEND, INDIANA, ASSIGNOR TO OLIVER CHILLED  
PLOW WORKS, OF SOUTH BEND, INDIANA.

## PLOWSHARE.

Application filed February 24, 1921. Serial No. 447,587.

To all whom it may concern:

Be it known that I, EDMUND J. LOWRY, a citizen of the United States, and a resident of South Bend, in the county of Saint Joseph and State of Indiana, have invented certain new and useful Improvements in Plowshares; and I do hereby declare the following to be a full, clear, and exact description of the invention, such as will enable others skilled in the art to which it appertains to make and use the same.

This invention relates to improvements in plow shares,—the object of the invention being to so construct a plow share as to enhance the strength, wearing qualities and longevity of the same.

A further object is to provide a plow share with a chilled cutting edge portion, which shall be uniform and in which the chilled portion shall extend not only an appreciable distance upwardly from the cutting edge per se, but which shall also extend an appreciable distance upwardly at both sides of the body metal of the share, this distance being governed by the varying of the analysis of the alloy giving the chill.

With these and other objects in view, the invention consists in certain novel features of construction as hereinafter set forth and pointed out in the claims.

In the accompanying drawings, Figure 1 is a view of a plow share embodying my invention, and Figure 2 is a transverse sectional view.

1 represents the body portion of the share which may consist of a suitable chilling iron alloy. The cutting edge portion of the share is chilled uniformly as indicated at 2. This chilled portion of the share extends an appreciable distance upwardly from the cutting edge, per se, and it also extends appreciable distances upwardly at respective sides of the body iron of the share as shown at 3, so that the body metal of the share will extend downwardly in V-shape (in cross section) into the chilled portion.

The formation of the chilled portion of the share as above described is brought about with the use of a chilling alloy and the upper limit of the chilled cutting edge portion is determined or governed by the analysis of the alloy used in molding the device. The desired results may be obtained with the use of an alloy consisting of iron having incorporated therein silicon from 2.40 to 2.70 per cent; sulphur from .06 to .15 per cent; phosphorus from .120 to .250 per cent and manganese from .50 to .85 per cent,—or the chilling mixture might be modified as follows: silicon 3.50 per cent; sulphur .06 to .15 per cent; manganese 1.0 per cent.

I have found that a plow share thus constructed is strong and durable and that such construction results in materially extending the efficient life of the share.

Having fully described my invention what I claim as new and desire to secure by Letters-Patent, is:

1. A plow share having a chilled cutting edge portion extending an appreciable distance beyond the cutting edge, per se, and the unchilled body metal of the share formed with a V-shaped portion extending into the chilled portion of the share, limited wholly by the analysis and shape of the cutting edge portion.

2. A plow share having a chilled cutting edge portion which extends an appreciable distance upwardly from the cutting edge, per se, and from one face to the other of the share, said chilled cutting edge portion having an approximately V-shaped portion occupied by unchilled body metal of the share.

In testimony whereof, I have signed this specification in the presence of two subscribing witnesses.

EDMUND JAMES LOWRY.

Witnesses:

ROSE B. MARBAUGH,  
JENNIE M. DAVIS.